

July 16, 1968

M. J. MONBALIU ET AL  
PHOTOGRAPHIC COLOR MATERIAL AND PROCESS UTILIZING  
5-PYRAZOLONE COLOR COUPLERS

3,393,071

Filed Oct. 8, 1964

2 Sheets-Sheet 1

FIG. 1 -



INVENTORS

M. J. Monbaliu  
A. H. DeCat  
R. K. Van Pouwakke,  
BY Watson, Cole, Grindle & Watson,  
ATTORNEYS

July 16, 1968

M. J. MONBALIU ET AL  
PHOTOGRAPHIC COLOR MATERIAL AND PROCESS UTILIZING  
5-PYRAZOLONE COLOR COUPLERS

3,393,071

Filed Oct. 8, 1964

2 Sheets-Sheet 2



BY *M. J. Monbaliu*  
*A. H. Decat*  
*R. K. Van Poucke*,  
*Watson, Cole, Grindle & Watson*,  
ATTORNEYS

1

3,393,071

PHOTOGRAPHIC COLOR MATERIAL AND  
PROCESS UTILIZING 5-PYRAZOLONE  
COLOR COUPLERS

Marcel Jacob Monbaliu and Arthur Henri De Cat, Mortsel-Antwerp, and Raphael Karel Van Poucke, Mechlin, Belgium, assignors to Gevaert Photo-Producten N.V., Mortsel, Belgium  
Continuation-in-part of application Ser. No. 314,807, Oct. 8, 1963. This application Oct. 8, 1964, Ser. No. 402,651

8 Claims. (Cl. 96—56.5)

ABSTRACT OF THE DISCLOSURE

5-pyrazolone color couplers having a urea linkage in combination with an alkyl group at the 3 position are described. The color couplers of the invention possess favorable spectral properties for use in positive and reversal color materials.

This invention relates to the manufacture of photographic color images.

The present application is a continuation-in-part of our application Ser. No. 314,807, filed Oct. 8, 1963, now 25 abandoned.

It is known that for the manufacture of a photographic image in a light-sensitive silver halide emulsion layer the exposed silver halide is developed to a silver image by means of an aromatic primary amino compound in the presence of a color coupler which by reaction with the oxidized developing substances forms a dye on the areas corresponding with the silver image.

In the subtractive three-color photography mostly a light-sensitive photographic color material is used comprising a red-sensitized, a green-sensitized and a blue-sensitive silver halide emulsion layer wherein on development by means of suitable color couplers, a cyan, a magenta and a yellow dye image are formed respectively.

As known, distinction should be made between color couplers for negative and positive materials e.g. with respect to the absorption spectrum of the dyes to be formed.

It is an object of the present invention to provide a method for the manufacture of photographic color images by means of color couplers which on color development with an aromatic primary amine as a developing substance form a magenta dye possessing favorable spectral properties for use in positive and reversal color material.

Another object of this invention is to provide photographic processing baths and photographic materials containing such color couplers.

These objects are accomplished by using, in the color development of a latent image of exposed silver halide, color couplers corresponding to the general formula:



wherein:

R is an alkyl radical, e.g. a lower alkyl radical such as an n-butyl radical or a higher alkyl radical preferably containing from 5 to 20 carbon atoms, e.g. an n-octadecyl radical, and

R<sub>1</sub> represents an unsubstituted aryl group, e.g. a phenyl group or a substituted aryl group, e.g. an alkyl-substituted phenyl group, an alkoxy-substituted phenyl group, a phenoxy-substituted phenyl group, a halogen-substituted phenyl group, an alkylsulfonyl-substituted phenyl group, an arylsulfonyl-substituted phenyl group,

2

a sulfamyl group and an N-substituted sulfamylphenyl group.

These color couplers can be prepared according to a method described in the U.S. patent application Ser. No. 314,594.

When the said color couplers do not contain a radical rendering the molecule fast to diffusion, they can be used in the developing solution. Preferably, however, they are incorporated in a non-migratory form into a light-sensitive silver halide emulsion layer or a non-light-sensitive water-permeable colloid layer, which is in direct contact with a light-sensitive layer or which is separated from it by a water-permeable layer. The color couplers used according to this invention are preferably rendered fast to diffusion by the introduction in their molecule of an acyclic aliphatic radical containing of from 5 to 20 carbon atoms in straight line.

New non-diffusing color couplers, which according to the present invention are preferably incorporated into the photographic material, have the following structure:



3

-4-

(6)



(7)



(8)



{9}



（五）



11



11



(13)



(15)



30

These color couplers may also be incorporated in a silver halide emulsion layer according to the methods of Mannes and Godowsky, U.S. patent specification 2,304,940 and of Jelleay and Vittum, U.S. patent specification 2,322,027. In the process of the latter patent specification the coupler is first dissolved in a water-insoluble high-boiling organic crystalloid material such as 1,2-dimethoxybenzene or dimethyl phthalate, and the solution is then dispersed in the silver halide emulsion.

40 According to a preferred embodiment for the manufacture of a light-sensitive color material according to the present invention, the 2-pyrazolin-5-one color couplers used in the present invention, which are rendered fast to diffusion by the introduction of a long aliphatic chain  
45 in their molecule, are dissolved in a water-miscible solvent such as ethanol and homogeneously mixed with the light-sensitive silver halide emulsion during the preparation of the latter. The silver halide emulsion normally contains the usual colloids such as gelatin, poly(vinyl alcohol),  
50 collodion or other natural or synthetic colloids suitable therefor.

The magenta-forming color coupler usually is added to the green-sensitized silver halide emulsion. According to a preferred embodiment this silver halide emulsion is applied as a second color coupler containing layer of a photographic multilayer color material. Such multilayer material usually comprises the following layers in the indicated sequence: a support, a red-sensitized silver halide emulsion layer containing a cyan-forming color coupler, a 55 green-sensitized silver halide emulsion layer containing a magenta-forming color coupler, a yellow filter layer mostly consisting of gelatin containing dispersed colloidal silver, and a blue-sensitive silver halide emulsion layer 60 containing a yellow-forming color coupler.

65 In the development of exposed photographic silver halide emulsion layers, using the couplers described above, any color-forming developer containing a primary amino group may be used. These include developers having two primary amino groups as well as those having one of  
70 the amino groups substituted or having substituents in the ring such as alkylphenylene-diamines. These compounds are usually used in the salt form such as the hydrochloride or the sulfate, which are more stable than the amines themselves. All of these compounds have an  
75 unsubstituted amino group, which enables the oxidation

products of the developer to couple with the color-forming compounds to form a dye.

Suitable developing substances are aromatic primary amino compounds such as p-phenylenediamine and derivatives thereof such as N,N-diethyl-N'-sulfomethyl-p-phenylenediamine and N,N-diethyl-N'-carboxymethyl-p-phenylenediamine.

One of the advantages of the couplers used according to our invention is that the dyes formed by coupling with an oxidized developing compound e.g. N,N-diethyl-p-phenylenediamine have an absorption curve with a very steep slope on the side of the long wave-lengths and with a very high transmission in the blue region of the visible spectrum.

The absorption curves represented in the accompanying drawings demonstrate clearly the favorable low transmission in the blue and the steep slope of the absorption curves of dyes obtained by means of color couplers used according to the present invention in respect of the transmission and the slope of the absorption curves of dyes obtained with color couplers of a type described in U.S. patent specification 2,369,489.

FIGURE 1 represents the absorption curves A and B of the dyestuffs that are formed by development with N,N-diethyl-p-phenylenediamine of the color couplers having respectively the following structural formulas:



FIGURE 2 represents the absorption curves C and D of the dyestuffs that are formed by development with N,N-diethyl-p-phenylene diamine of the color couplers having respectively the following structural formulas:



and



The following examples illustrate the invention.

*Example 1*

To  $\frac{1}{2}$  kg. of a green-sensitive silver halide emulsion containing 0.0950 mol of silver chloride are added 10 g. of the color coupler having the structural Formula 4 dissolved in a mixture of 40 ml. of 1 N sodium hydroxide, 32 ml. of isopropanol and 32 ml. of distilled water. After addition of the usual additives such as hardeners, wetting agents, stabilizers and the necessary amount of distilled water to obtain 1 kg. of emulsion, the latter is coated onto a cellulose triacetate support and dried.

After exposure with green light through a grey wedge, the photographic material is developed for 7.5 min. at 20° C. in a color-developing bath of the following composition:

|                                       |      |
|---------------------------------------|------|
| N,N-diethyl-p-phenylenediamine hydro- | 3    |
| chloride                              | g    |
| Sodium hexametaphosphate              | 1    |
| Hydroxylamine hydrochloride           | 1.2  |
| Anhydrous sodium sulfite              | 4    |
| Anhydrous sodium carbonate            | 50   |
| Potassium bromide                     | 2.5  |
| Water up to                           | 1000 |

The developed material is rinsed with water for 30 sec. at 18° C. and fixed for 4 min. at 20° C. in a fixing bath of the following composition:

|                                   |      |
|-----------------------------------|------|
| Sodium thiosulfate-5-water        | 300  |
| Anhydrous potassium metabisulfite | 12   |
| Acetic acid (99%)                 | 12   |
| Borax                             | 20   |
| Potassium alum                    | 15   |
| Water up to                       | 1000 |

Next, the material is rinsed again for 6 min. at 18° C. and treated for 4 min. in a bleaching bath of the following composition:

|                      |      |
|----------------------|------|
| Potassium dichromate | 5    |
| Potassium bromide    | 20   |
| Potassium alum       | 40   |
| Sodium bisulfite     | 0.6  |
| Water up to          | 1000 |

After bleaching, the material is rinsed for 4 min. at 18° C. and fixed again in the fixing bath composed as described above. After a further rinsing for 6 min. at 18° C. the material is stabilized in the following stabilizing bath:

|                                                   |      |
|---------------------------------------------------|------|
| Anhydrous sodium carbonate                        | 10   |
| Disodium salt of ethylenediamine tetraacetic acid | 2    |
| Paraformaldehyde                                  | 5    |
| Water up to                                       | 1000 |

A magenta wedge-image having an absorption maximum at 525 m $\mu$  is obtained.

*Example 2*

A similar silver halide emulsion as described in Example 1, wherein the color coupler is replaced by a same amount of the color coupler having the structural Formula 2 dissolved in a mixture of 80 ml. of 0.5 N sodium hydroxide, 80 ml. of isopropanol and 80 ml. of distilled water. After the addition of the usual additives such as hardeners, wetting agents, stabilizers and the necessary amount of distilled water to obtain 1 kg. of emulsion, the latter is coated onto a cellulose triacetate support and dried. After exposure and further processing as described in Example 1, a magenta colored image is obtained having an absorption maximum of 530 m $\mu$ .

*Example 3*

To  $\frac{1}{2}$  kg. of a green-sensitive silver halide emulsion containing 0.0950 mol of silver chloride are added 10 g. of the color coupler having the structural Formula 4, dissolved in a mixture of 40 ml. of 1 N sodium hydroxide,

32 ml. of isopropanol and 32 ml. of distilled water. After addition of the usual additives such as hardeners, wetting agents, stabilizers and the necessary amount of distilled water to obtain 1 kg. of emulsion, the latter is coated to form part of a multilayer photographic color material. The multilayer photographic material consists in the indicated sequence of an antihalation layer, a support, a gelatin subbing layer, a red-sensitive silver halide emulsion layer containing a cyan-forming color coupler, a gelatin interlayer, a layer of a green-sensitive silver halide emulsion prepared as described above, a yellow filter layer, a blue-sensitive silver halide emulsion layer containing a yellow-forming color coupler, and at least one gelatin overcoat as antistress layer.

The multilayer color material is exposed through a color negative and further processed as described in Example 1. A positive color image is obtained.

We claim:

1. A method of producing a magenta colored photographic image in a silver halide emulsion layer, which comprises exposing the layer and developing the layer with an aromatic primary amine in the presence of a coupler compound having the following general formula:



in which R is an alkyl radical containing from 4 to 20 carbon atoms, and R<sub>1</sub> is an aryl radical.

2. A method of producing a magenta colored photographic image in a silver halide emulsion layer, which comprises exposing the layer and developing the layer with an aromatic primary amine in the presence of a coupler compound having the following general formula:



in which  $R'$  is a higher alkyl radical containing from 5 to 20 carbon atoms, and  $R_1$  is an aryl radical.

3. A method of producing a magenta colored photographic image in a silver halide emulsion layer, which comprises exposing the layer and developing the layer with an aromatic primary amine in the presence of a coupler compound having the following general formula:



in which R is an alkyl radical containing from 4 to 20 carbon atoms, and R' is a phenyl radical.

4. A color-forming photographic developer comprising a primary aromatic amino developing agent and a coupler compound having the following general formula:



in which  $R''$  is a lower alkyl radical, and  $R_1$  is an aryl radical.

10 5. A color-forming photographic developer comprising a primary aromatic amino developing agent and a coupler compound having the following general formula:



in which  $R''$  is a lower alkyl radical, and  $R'_1$  is a phenyl radical.

6. A photographic emulsion for preparing a photographic element for forming colored images comprising a water-permeable colloid as carrier for light-sensitive silver halide and a color coupler having the general formula:



in which R is an alkyl radical containing from 4 to 20 carbon atoms, and R<sub>1</sub> is an aryl radical.

30 7. A photographic element containing at least one silver halide emulsion layer and containing in non-migratory form a coupler compound having the following general formula:



40 in which R is an alkyl radical containing from 4 to 20 carbon atoms, and R<sub>1</sub> is an aryl radical.

8. A photographic element containing at least one silver halide emulsion layer, which contains a coupler compound having the following general formula:



50 in which  $R'$  is an alkyl radical containing from 5 to 20 carbon atoms, and  $R_1$  is an aryl radical.

### References Cited

UNITED STATES PATENTS

- 2,369,489 2/1945 Porter et al. ----- 96-100  
3,161,512 12/1964 Greenhalgh ----- 96-100

J. TRAVIS BROWN, *Primary Examiner.*